

March 8, 1932.

J. L. STEVENS

1,848,396

CONCENTRATION OF ORES

Filed Aug. 27, 1930

5 Sheets-Sheet 1



FIG. 1

INVENTOR

James L. Stevens

BY Arthur P. Knapp and  
Alfred W. Knapp  
ATTORNEYS

March 8, 1932.

J. L. STEVENS

1,848,396

CONCENTRATION OF ORES

Filed Aug. 27, 1930

5 Sheets-Sheet 2



FIG. 2

INVENTOR

James L. Stevens

BY Arthur P. Knapp and

Alfred W. Knapp

ATTORNEYS

March 8, 1932.

J. L. STEVENS

1,848,396

CONCENTRATION OF ORES

Filed Aug. 27, 1930

5 Sheets-Sheet 3



INVENTOR  
James L. Stevens  
BY Arthur P. Knapp and  
Alfred W. Knapp  
ATTORNEYS

FIG. 3

March 8, 1932.

J. L. STEVENS

1,848,396

CONCENTRATION OF ORES

Filed Aug. 27, 1930

5 Sheets-Sheet 4



FIG. 4

INVENTOR  
James L. Stevens  
BY Arthur P. Wright and  
Alfred W. Wright  
ATTORNEYS

March 8, 1932.

J. L. STEVENS

1,848,396

CONCENTRATION OF ORES

Filed Aug. 27, 1930

5 Sheets-Sheet 5



FIG. 5

INVENTOR

James L. Stevens  
BY Arthur P. Knights and  
Alfred W. Knights  
ATTORNEYS

## UNITED STATES PATENT OFFICE

JAMES L. STEVENS, OF HAYDEN, ARIZONA

## CONCENTRATION OF ORES

Application filed August 27, 1930. Serial No. 478,135.

This invention relates to the concentration of copper bearing ores, and has for its object certain provisions for improved economic recovery of the valuable constituents of complex ores containing sulphide and non-sulphide copper minerals.

In general, clean sulphide copper minerals are readily amenable to recovery by the customary methods employed in the modern flotation processes, while certain non-sulphide copper minerals are quite refractory and usually constitute the major portion of the tailings losses.

The non-sulphide copper minerals are generally referred to as "oxide", and include various oxides, carbonates, silicates, etc. of copper. Hereinafter the term "oxide" shall be employed to include the above mentioned class of non-sulphide copper minerals which readily form copper sulphate by reaction with dilute sulphuric acid.

Many copper bearing ores, requiring concentration by flotation, contain an appreciable amount of oxide copper together with copper sulphides and gangue sulphides such as pyrite, and in the concentration of such ores, it is frequently desirable to reject a substantial amount of the pyrite with the tailings. The present invention is particularly adapted to the treatment of such complex ore, and the specific example given herein is directed to an ore of this type. However, the invention in its broadest aspect contemplates the treatment of any copper oxide bearing ore.

The present invention, briefly described, consists of subjecting the total ore (crushed to a suitable size), or portions of such ore, to an acid leaching operation (using sulphuric acid or other suitable acid) to dissolve the oxide copper, classifying the leached ore (including the solution or liquor formed during leaching) so that the dissolved copper is collected with the relatively fine slime portion of the ore, precipitating the dissolved copper in the slime pulp by action of a suitable precipitant such as metallic iron, subjecting the slime pulp containing the copper precipitate to flotation to produce a copper bearing concentrate, and subjecting the coarse washed

portion of the ore to any suitable separate treatment.

In general, the major portion of the oxide copper of the ore is obtained as dissolved copper in the slime pulp, while the major portion of the sulphide copper, and of the pyrite when present, is collected in the coarser portion.

By classifying the leached ore, the dissolved copper may be concentrated in a relatively strong pulp solution which enables the subsequent treatment to be carried out very efficiently. Classifying also permits the clean washed coarse portion of the ore to be subjected to any method of disposal or treatment to which it is best adapted. For example, the coarse classified portion of an ore containing copper sulphide minerals and pyrite may be crushed or ground to a suitable size and subjected to flotation treatment adapted to selectively concentrate the copper bearing minerals from the free pyrite.

Methods for precipitating dissolved copper in an ore pulp, followed by floatation for its recovery together with the natural sulphides of the ore are old in the art. For example, U. S. Pat. No. 1,268,940 issued to B. H. Dosenbach discloses such a process. However, prior to my investigations, no provision had been made for concentrating the dissolved copper with the fine slime portion of the ore pulp for separate subsequent precipitation and recovery by floatation.

The advantages of the present invention are shown in various ways: in some cases by reducing the amount of acid required; in some cases by effecting markedly better recoveries of the copper; in some cases by permitting different and separate treatment of the various classified products; and in some cases by markedly reducing the time and cost of the recovery of the copper in the floatation operation.

According to a preferred embodiment of the invention, the separate treatment of the coarse portion of the ore, after separating the slime pulp and dissolved copper therefrom and washing the coarse material, consists in grinding these coarse sands sufficiently fine for treatment by floatation, and then

subjecting this ground material to a separate flotation operation. The separate flotation treatment of the original slime pulp containing the precipitated copper, and of the ground sands, leads to several practical advantages, by reason of the fact that these two materials differ considerably in composition and also in physical characteristics, and consequently require somewhat different conditions for maximum efficiency of concentration by flotation. For example, I find it advantageous in some cases to maintain an acid condition in the slime pulp during flotation treatment thereof, and an alkaline condition in the pulp obtained by grinding the coarse material, during its flotation treatment. Furthermore, different collectors or other flotation reagents may be used, which are particularly adapted to the concentration of copper in the two pulps.

Other advantages will be obvious from the following description and from the results of tests as given hereinafter.

Figs. 1, 2, 3, 4 and 5 of the accompanying drawings are flow sheets showing various schemes or arrangements which may advantageously be employed in carrying out the present invention. In these drawings the apparatus employed, or the operations involved, are indicated by legends, as are also the materials introduced into the process, the materials, delivered from each stage of the process to the next, and the final products obtained, so that the drawings are self-explanatory. However, the following general remarks may be made regarding the schemes illustrated in the several figures.

Fig. 1 illustrates the invention in its simplest form and corresponds substantially to the general description of the invention given above.

Fig. 2 illustrates the embodiment of the invention mentioned above, in which the treatment of the coarse portion of the ore obtained from the classifying operation consists in grinding this material and then subjecting it to a separate flotation operation. In this case the slime pulp containing dissolved copper, delivered from the classifying apparatus, is subjected to the same treatment as in Fig. 1, except that, by way of example, I have indicated the use of metallic iron as a precipitant for the copper. The coarse sands, after washing, and after addition of suitable conditioning agents thereto for assisting in subsequent concentration of the copper bearing constituents by flotation, are ground to proper fineness and are then subjected to a flotation operation in the presence of suitable reagents, to produce a separate copper bearing concentrate.

A somewhat more elaborate scheme of treatment is illustrated in Fig. 3. In this case the crushed ore is first screened, and the oversize and undersize materials are leached

separately. According to the particular arrangement shown, the oversize material is leached with acid to dissolve oxide copper therefrom, and the resulting liquor, containing some dissolved copper but still containing excess acid, is separated from the coarse solids and is used to dissolve a further quantity of oxide copper from the undersize material. The leached undersize material, together with the leaching liquor, is classified and washed, to produce a washed sand product and a product consisting, as before, of the slimes together with the liquor containing dissolved copper. The leached coarse solids from the oversize material are washed, and the wash water from this operation may advantageously be used to furnish part of the water required in the classifying and washing of the leached undersize material. The washed sands obtained from the leached undersize material are combined with the leached and washed coarse solids from the oversize material, suitable conditioning agents are added, and the materials are ground and subjected to flotation to obtain one copper bearing concentrate, while the mixed product of slimes and liquor containing dissolved copper is subjected to the same treatment as before, involving precipitation of the copper and subsequent flotation, to obtain another copper bearing concentrate.

In some cases, in order to effect the desired separation of slimes, a lower percentage of solids must be maintained in the classifying operation than is desirable in the subsequent treatment of the slime pulp. In such cases a scheme such as shown in Fig. 4, which provides for thickening the classified slime pulp and returning the overflow liquor from the thickener to the classifier in closed circuit, may be advantageously employed. The scheme shown in Fig. 4 also provides for the return of part of the thickener overflow liquor to the leaching apparatus in order to further reduce the amount of fresh water added during the leaching and classifying operations. Fig. 4 also provides for wetting the ore, if desirable, with fresh water prior to treatment in the leaching apparatus and also provides fresh water for washing the coarse material in the classifying and washing apparatus. The combined amounts of fresh water, going with the slime pulp from the classifier, added prior to classification and used in washing the coarse material should be regulated to equal the amount discharged with the thickened slimes from the thickener.

The pre-wetting of the crushed ore with water prior to applying the leaching acid is advantageous in hindering absorption of the acid solution by the clean ore particles, in cases where the ore is very dry and the major portion of the copper is present in the form of sulphide, with the oxidized copper occurring chiefly at the surfaces of the ore.

particles. On the other hand, if the major portion of the copper content of the ore is present as oxide and more or less disseminated throughout the ore, the acid solution may be advantageously applied to the dry ore in order to promote absorption and contact of the acid.

I will now describe an application of my invention to one particular ore and the results obtained, it being understood, however, that this is given only as an example and that the invention is not restricted to the use of the specific reagents, nor to the particular proportions given below. Fig. 5 represents the flow sheet of this particular application of the invention.

#### *Treatment of crude ore*

A sample of crude ore (crushed to approximately minus three-quarter inch size and containing ore material of various degrees of fineness ranging from three-quarter inch size to fine material of a clay-like nature) consisting chiefly of schist and porphyry rock containing disseminated minerals of copper and iron; the copper minerals consisting of chalcocite and small amounts of other sulphides such as chalcopyrite, etc., and various oxides such as chrysocolla, malachite, sulphate, etc., and the iron being in the form of oxides and sulphides but chiefly in the form of pyrite extensively intercrystallized with the chalcocite), was subjected to an acid leach using sulphuric acid at the rate of six pounds per ton of ore in conjunction with just sufficient water to completely cover the ore and give the mass a semi-fluid consistency. The ore was given about ten minutes contact with the strong acid solution with intermittent stirring, after which sufficient water was added to permit separating the fine slime pulp by decanting and draining same, with the liquor containing the dissolved copper, from the coarse material. The coarse material was finally washed with fresh water and all wash waters added to the slime pulp. The total volume of leaching solution and wash water used in leaching, classifying and washing the ore was equivalent to the rate of 0.66 of a ton of water per ton of original ore.

#### *Original crude ore assay*

|              |               | Per cent |
|--------------|---------------|----------|
| Copper       | Oxide-----    | 0.17     |
|              | Sulphide----- | 0.75     |
|              | Total-----    | 0.92     |
| Iron (total) | -----         | 4.31     |

#### *Products of classification*

|                      | % Weight of original ore | Copper per cent |          |       | Total iron % |
|----------------------|--------------------------|-----------------|----------|-------|--------------|
|                      |                          | Oxide           | Sulphide | Total |              |
| Coarse material..... | 85.6                     | .052            | .775     | 0.827 | 4.47         |
| Slimes.....          | 14.4                     | *.87            | .60      | 1.47  | 3.34         |

65 \* Leached copper in solution shown as "oxide" per cent of ore slimes.

The above analysis of the products of classification show that about 73.8% of the oxide copper is concentrated with the slime material, and about 88.5% of the copper sulphide together with about 88.8% of the iron is retained with the coarse material. The amount of pyrite in each of the above products of classification was not determined. However, with this particular ore, it is known that, in general, the major portion of the iron in the coarse classified material is in the form of sulphide (pyrite), and that the major portion of the iron in the classified slimes is in the form of oxide. It is thus evident that the classification results in collecting the major portion of the copper sulphide minerals and pyrite with the relatively coarse portion of the ore material.

#### *Treatment of coarse material*

The coarse material was crushed by rolls to approximately minus ten mesh. Lime, at the rate of one pound per ton of ore, was then added and the ore made up into a pulp by addition of water. The ore pulp was then classified into sands and (secondary) slimes by washing out the fines produced by the rolls. Lime at the rate of three pounds per ton of original coarse material was added to the classified sands and the sands ground (wet) in a pebble mill to a suitable size for flotation treatment. The classified (secondary) slime pulp was thickened and lime at the rate of one pound per ton of original coarse material added. Butyl xanthate at the rate of 0.05 pound per ton of original coarse material, in a crude aqueous solution containing approximately one part of sodium thio-carbonate to 2.34 parts of sodium butyl xanthate, was added to the thickened (secondary) slime pulp and allowed two hours' contact. The ground sand pulp and the (secondary) slime pulp were then combined and subjected to flotation treatment to produce a copper bearing concentrate; pine oil being employed in the flotation operation as needed to produce the required froth.

#### *Treatment of leached slimes*

The acid slime pulp containing dissolved copper was allowed to stand about three hours and was then placed in a grinding mill charged with a mixture of steel balls and pebbles and ground until the dissolved copper was precipitated by action of the iron contained in the steel balls. After precipitating the dissolved copper, the slime pulp containing same was taken from the mill and subjected to flotation treatment to recover, as a flotation concentrate, both the precipitated and natural sulphide copper contained in this pulp.

The mineral collecting agent employed in the flotation operation consisted of an organic compound formed by reaction between potas-

sium ethyl xanthate and sulphur monochloride; having the formula



5

This new flotation agent is described in my pending patent application Ser. No. 332,741. Any suitable collecting agent may of course be employed. However, a collecting agent of this type is very attractive for this particular type of ore pulp because its effectiveness is not destroyed by acid or mineral salts that might be present.

The above described collecting agent was employed at the rate of 0.26 pound per ton of slimes; 50% being added to the pulp during precipitation and 50% just ahead of flotation. Smaller amounts of this reagent have been found very effective.

20 Pine oil was employed to give the required amount of froth during flotation.

*Flotation results*

| 25 | Test No.                                                                                    | Tailings |       | Concentrates |      |        |
|----|---------------------------------------------------------------------------------------------|----------|-------|--------------|------|--------|
|    |                                                                                             | % Cu     | % Fe  | % Cu         | % Fe | % Ins. |
| 30 | 1. Classified coarse material.....                                                          | .080     | 3.31  | 16.4         | 30.7 | 11.7   |
|    | 2. Classified slime material.....                                                           | .100     | *2.69 | 29.4         | 31.4 | 11.2   |
|    | Combined results of tests #1 and #2.....                                                    | .083     | 3.23  | 18.2         | 30.8 | 11.6   |
| 35 | 3. Standard bulk flotation results on same ore without special leaching treatment.....      | .175     | 1.99  | 10.5         | 34.0 | 9.7    |
|    | 4. Standard selective flotation results on same ore without special leaching treatment..... | .195     | 3.00  | 17.5         | 30.8 | 8.8    |

\* This result includes part of the iron in the form of iron salts from the metallic iron precipitant.

The percentage of solids contained in the slime pulp may be varied considerably according to the nature of the slimes of the ore treated. For slimes of a clay-like nature a pulp containing 15 to 20 per cent solids has been found satisfactory, both in the precipitating and flotation operations. In general, I prefer to maintain a high percentage of solids in the slime pulp in order to concentrate the dissolved copper in a small volume of pulp. However, the slime pulp should be quite fluid, and not contain a percentage of solids sufficiently high to hinder precipitation or flotation.

The presence of free acid in the slime pulp aids precipitation of the dissolved copper. In general, I prefer to apply sufficient acid to the total ore in the original leaching operation to supply free acid during precipitation. However, in case the initial acid should be exhausted in the leaching operation, the desired amount may be added prior to precipitation.

In some cases the presence of free acid in the slime pulp during flotation is advantageous, and in case the initial acid added for leaching and precipitation should be exhausted prior to the flotation treatment, fresh acid

may be added at the flotation machine to supply the desired amount in the flotation circuit.

A ball mill containing steel balls has been found satisfactory as an apparatus for precipitating the dissolved copper. Any other suitable apparatus and/or precipitant may, however, be employed. I have also found that satisfactory precipitation may be accomplished by agitating the slime pulp, containing the dissolved copper, with sponge or pulverized iron.

Any suitable flotation reagents and type of flotation apparatus may be employed for recovery of a copper bearing concentrate from the slime pulp. If the type of collecting agent described in the foregoing specific example for treatment of the slime pulp be employed, it is not necessary to alter the conditions of the pulp from the precipitating operation, for flotation treatment, as this type of reagent functions very effectively in an acid or neutral pulp and is not destroyed by mineral salts, such as, for example, ferrous sulphate formed during precipitation. This type of collecting agent, however, may in some cases require more agitation for proper dispersion throughout the pulp than is provided for in certain types of flotation apparatus, and in such cases the pulp may be advantageously pre-agitated with the reagent to effect proper dispersion prior to flotation treatment.

I claim:

1. A method of concentrating ores which comprises subjecting an ore, containing oxide copper minerals, to a leaching operation, classifying the leached ore so as to collect the dissolved copper with the slime portion of the ore, precipitating the dissolved copper in the slime pulp and subjecting the slime pulp to a flotation operation for separation of a copper bearing concentrate.

2. A method of concentrating ores which comprises subjecting an ore, containing oxide copper minerals, to a leaching operation in the presence of sulphuric acid, classifying the leached ore so as to collect the dissolved copper with a slime pulp containing the relatively fine portion of the ore, precipitating the dissolved copper in the slime pulp as a metallic precipitate and subjecting the pulp to a flotation operation for separation of a copper bearing concentrate.

3. A method of concentrating ores which comprises subjecting an ore, containing oxide copper minerals, to a sulphuric acid leaching operation, classifying the leached ore so as to collect the dissolved copper with slime pulp containing the relatively fine portion of the ore, precipitating the dissolved copper in the slime pulp as a metallic precipitate by action of metallic iron and subjecting the pulp to a flotation operation for separation of a copper bearing concentrate.

4. The improvement in the concentration of ores which comprises classifying a leached ore pulp containing dissolved copper so as to collect the dissolved copper with a pulp containing the relatively fine portion of the ore material and obtain a separate relatively coarse portion of the ore, precipitating the dissolved copper in the presence of the fine portion of the ore, subjecting the pulp containing the copper precipitate to a flotation operation for separation of a copper bearing concentrate, and treating the separated relatively coarse portion of the ore separately. 5. The improvement in concentrating ores which comprises classifying an ore material, leached by action of sulphuric acid and containing dissolved copper, so as to collect the dissolved copper with a pulp containing the relatively fine portion of the ore material and obtain a separate product containing the relatively coarse portion of the ore material, precipitating the dissolved copper as a metallic precipitate by action of metallic iron, subjecting the pulp containing the metallic copper precipitate to a flotation operation for separation of a copper bearing concentrate, and subjecting the separated relatively coarse portion of the ore material to separate treatment. 6. A method of concentrating ores which comprises subjecting an ore material containing oxide and sulphur copper minerals to a leaching operation, classifying the leached ore so as to collect the dissolved copper with a pulp containing the relatively fine portion of the ore and obtain a separate relatively coarse portion of the ore material, precipitating the dissolved copper in the presence of the fine portion of the ore material, subjecting the pulp containing the copper precipitate to a flotation operation for separation of a copper bearing concentrate, grinding the separated relatively coarse portion of the ore material to a suitable size for flotation treatment, and subjecting the ground coarse portion of the ore material to a separate flotation operation for separation of a copper bearing concentrate. 7. A method of concentrating ores which comprises subjecting an ore material containing oxide and sulphur copper minerals to a sulphuric acid leaching operation, classifying the leached ore so as to collect the dissolved copper in a pulp containing the relatively fine portion of the ore material and obtain a separate relatively coarse portion of the ore material, applying metallic iron to the pulp comprising the fine portion of the ore material to precipitate the dissolved copper, subjecting the pulp containing the metallic copper precipitate to a flotation operation to separate a copper bearing concentrate, the pulp being in an acid condition during flotation, grinding the relatively coarse portion of the ore material to a suitable size for flotation treatment, and subjecting the ground coarse portion of the ore material to a separate alkaline flotation operation for separating a copper bearing concentrate. 8. A method of concentrating ores which comprises subjecting material containing oxide and sulphur copper minerals together with pyrite to a sulphuric acid leaching operation, classifying the leached material so as to collect the dissolved copper in a pulp containing the relatively fine portion of the material and collect the major portion of the copper sulphide minerals and pyrite with the relatively coarse portion of the material, applying metallic iron to the pulp comprising the fine portion of the material to precipitate the dissolved copper, subjecting the pulp containing the metallic copper precipitate to a flotation operation to separate a copper bearing concentrate, grinding the relatively coarse portion of the material in the presence of added lime, and subjecting the ground pulp to a separate flotation operation for separating a copper bearing concentrate from pyrite and other gangue constituents.
- 80
- 85
- 90
- 95
- 100
- 105
- 110
- 115
- 120
- 125
- 130

In testimony whereof I have hereunto subscribed my name this 21st day of August, 1930.

JAMES L. STEVENS. 110